

Patented Sept. 14, 1926.

1,600,156

# UNITED STATES PATENT OFFICE.

WILLIAM WHYTE, OF EDINBURGH, SCOTLAND.

## METHOD OF DECORATIVE PAINTING.

No Drawing. Original application filed August 27, 1924; Serial No. 734,524, and in Great Britain September 22, 1923. Divided and this application filed April 17, 1925. Serial No. 23,966.

This invention has for its object to produce improved decorative effects in low colour relief on walls or other surfaces by the application of an improved separating paint forming the subject of my concurrent patent application Serial No. 734,524 and filed 27th August, 1924, of which this application is a division and having the inherent quality of separating or producing natural irregular designs in relief on the wall or other surface without requiring the previous application to the surface of an undercoat of special composition.

The aforesaid separating paint consists of the following ingredients in the following approximate proportions: 80 to 100 lbs. of Paris white (sifted and dry), 4 to 6 lbs. of stucco, 7 to 9 lbs. lithopone, 6 to 8 lbs. hard and soft strong gums in suitable proportions such as 4½ lbs. of gum arabic to 1½ lbs. of gum tragacanth, each dissolved in just sufficient water, 1½ lbs. of cream of tartar and 12½ lbs. of water are mixed and finely ground in a roller mill or the like. In a separate vessel I mix 5½ lbs. of finely ground zinc oxide with 5½ lbs. of linseed oil (fire-boiled), also known as Dutch stand oil, 2½ lbs. paraffin oil, 2½ lbs. of pale boiled linseed oil with a suitable drier. I then incorporate the whole together by thorough mixing and the material is then ready for use.

The improved separating paint can be applied to any dry surface which has been previously rendered non-absorbent such as by means of one or two coats of ordinary oil paint, and can be applied over a dry oil-painted surface of any colour, without the previous application of an undercoat of special composition. The separation of my improved paint on the surface to which it is applied, reveals the ground colour as part of the finish, thus giving a two colour effect when applied to a plain painted surface.

If higher relief is desired, two coats of my improved separating paint may be applied to the surface, using an intermediate coat of oil paint.

The decorative effects in low colour relief obtained by my improved separating paint can be glazed, scumbled or wiped. Various irregular designs in relief, such as loops, globules and other markings, can be obtained by varying the relative proportion of water and oil in my improved separating

paint according to the result desired. Should regularity of the surface design be desired, the surface may be stippled slightly.

The improved separating paint can be applied to the surface by means of a brush 60 and the decorative surface so produced may be scumbled with metallic effects by the use of gold or other bronzes in any suitable medium.

The improved separating paint can be 65 tinted with oil colour or other colouring substances or it may be glazed over with suitable colours, scumbled and wiped in the usual manner according to the colour scheme in use.

A gold, bronze or like background can be imparted to the decorative design by rubbing lightly over the following day or later, according to temperature, with a flannel or other suitable pad dipped in the gold, bronze 75 or like powder. The gold, bronze or like background is produced by reason of the fact that the raised parts of the design produced by my improved separating paint dry at a quicker rate than other parts and the powder, when rubbed over the design, adheres to the slower drying parts of the design resulting in a metal ground with a pattern either white or otherwise according to whether the improved separating paint is 80 tinted or not before application to the surface.

To produce a scumble glaze I prefer to use a composition of pale varnish, bleached boiled oil and paraffin in equal quantities 90 with a suitable liquid drier and the necessary pigments. This gives a refined degree of colour and protects the bronze portion from atmospheric influences.

An effect of free-hand design of a serpentine or other regular or irregular character may be obtained by first applying my improved separating paint to a dry oil-painted ground and, immediately thereafter, before the first coat is dry, applying thinned-out 95 separating paint with a brush or the like in a series of S-shapes, loops or other regular or irregular figures, the thinning-out of the separating paint being effected by the addition of more water. The thinner paint 100 separates with more energy and produces a non-repeating pattern of serpentine or other regular or irregular character wherein the pattern produced varies with each S-shape or other figure adopted in the applica- 110

tion of the brush. When dry, the surface may be scumbled or glazed e. g. glazed with one-third pale varnish, one-third pale boiled oil and one third paraffin with a drier and suitable pigment. While the glaze is wet, it may be combed with a piece of felt or like material notched on edge and drawn perpendicularly over the work, giving a jaspé effect to the background portion of the design.

10 An irregular non-repeating tree or foliage pattern may be executed with my improved separating paint by applying the brush-work in slightly overlapping form, such as criss-cross-wise or after the manner of overlapping herring-bone pattern. When dry, a coat of ordinary black or other dark oil paint is applied over the separating paint which, when dry, may be given one coat of varnish. After drying, the surface may be scumbled with a gold paint scumble or any other suitable scumble which, being wiped into the loops formed by the separation of the paint on the flat surface, gives the effect of overhanging foliage, which can be further enhanced by the use of green, brown or other glazes.

Claims:

1. The method of producing an improved decorative effect in low colour relief upon a surface, which consists in applying a paint composed of Paris white, stucco, lithopone, gums, cream of tartar and water incorporated with zinc oxide, Dutch stand oil, paraffin oil, boiled linseed oil and a drying agent directly to the surface when the surface is in a dry state.

2. The method of producing an improved decorative effect in low colour relief upon a surface, which consists in rendering the surface non-absorbent by the application of an oil paint, allowing the surface so painted to dry and thereafter directly applying a paint composed of Paris white, stucco, lithopone, gums, cream of tartar and water incorporated with zinc oxide, Dutch stand oil, paraffin oil, boiled linseed oil and a drying agent to the oil painted surface.

3. The method of producing an improved decorative effect in low colour relief upon a

surface, which consists in applying a paint composed of Paris white, stucco, lithopone, gums, cream of tartar and water incorporated with zinc oxide, Dutch stand oil, paraffin oil, boiled linseed oil and a drying agent directly to the surface when the surface is in a dry state and thereafter rubbing over the surface with a decorative metallic powder.

4. The method of producing an improved decorative effect in low colour relief upon a surface, which consists in applying a paint composed of Paris white, stucco, lithopone, gums, cream of tartar and water incorporated with zinc oxide, Dutch stand oil, paraffin oil, boiled linseed oil and a drying agent directly to the surface when the surface is in a dry state, whereby the paint separates, forming irregular markings, and varying the markings by regulating the relative proportion of water and oil in the paint.

5. The method of producing an improved decorative effect in low colour relief upon a surface, which consists in applying a paint composed of Paris white, stucco, lithopone, gums, cream of tartar and water incorporated with zinc oxide, Dutch stand oil, paraffin oil, boiled linseed oil and a drying agent directly to the surface when the surface is in a dry state and finally treating the surface with a scumble glaze consisting of pale varnish, bleached boiled oil, paraffin, a liquid drying agent and pigments.

6. The method of producing an improved decorative effect in low colour relief upon a surface, which consists in applying a paint composed of Paris white, stucco, lithopone, gums, cream of tartar and water incorporated with zinc oxide, Dutch stand oil, paraffin oil, boiled linseed oil and a drying agent directly to the surface when the surface is in a dry state and finally treating the surface with a scumble glaze consisting of pale varnish, bleached boiled oil and paraffin in equal quantities with a liquid drying agent or pigments.

In testimony whereof I affix my signature.

WILLIAM WHYTE.